

## UNITED STATES PATENT OFFICE

2,639,266

LUBRICATING GREASE COMPRISING A  
COMPLEX ESTER BASE AND SODIUM  
MYRISTATE

John P. Dilworth and Charles H. Culnane, Fishkill, N. Y., assignors to The Texas Company, New York, N. Y., a corporation of Delaware

No Drawing. Application April 7, 1951,  
Serial No. 219,892

10 Claims. (Cl. 252—42)

1

The present invention relates to a wide temperature range ball and roller bearing grease. More particularly it relates to a lubricating grease composition comprising as the oil component a complex polyester of the type obtained by esterifying a dicarboxylic acid with both a monohydric alcohol and a dihydric ether alcohol and a thickening agent comprising sodium myristate.

There is a rapidly growing demand, particularly by aircraft engineers and by the manufacturers of prepacked bearings, for lubricating greases which will provide good lubrication for anti-friction bearings over a wide temperature range, such as from about  $-50^{\circ}$  F. or lower up to about  $200^{\circ}$  F. or higher. Ball and roller bearing greases of the usual type, comprising mineral oil fractions thickened with various fatty acid soaps, are unsuitable for use under conditions involving wide variations in temperature because of the changes in texture and consistency which they undergo with changes in temperature. Recently it has been found that all or a part of the mineral oil base of such greases may be replaced by non-hydrocarbon oils such as various esters, polymerized ethers and the like, with considerable improvement in the low temperature torque characteristics of the greases. The esters of aliphatic dibasic acids have been recommended particularly for this purpose because of their high boiling points, low pour points and high viscosity indexes.

However, it has been found that the improved low temperature characteristics of these so-called synthetic greases of the types heretofore proposed are obtained at the expense of other lubricating properties. In particular they are unsuitable for the long time lubrication of anti-friction bearings at ordinary or elevated temperatures.

It is a principal object of this invention to provide an improved lubricating grease for the lubrication of anti-friction bearings over a wide temperature range. A further object is to provide a synthetic base lubricating grease of greatly extended service life.

In accordance with our invention a grease having superior lubricating properties for the long time lubrication of anti-friction bearings over a wide temperature range comprises an oleaginous base and a thickening agent comprising

2

ing in major proportion sodium myristate, said oleaginous base comprising in substantial proportion at least a high molecular weight complex linear polyester of lubricating characteristics containing an ether linkage, which may be obtained by esterifying a dicarboxylic acid with both a monohydric alcohol and a dihydric ether alcohol. Suitable compounds of this character may be represented by the general formula



wherein R is an aliphatic ether group containing from 4 to 12 carbon atoms, R<sub>1</sub> is an alkyl group containing from 1 to 12 carbon atoms, R<sub>2</sub> is an alkyl group containing from 1 to 12 atoms and x is an integer from 1 to 5. Preferably R is an aliphatic ether group containing from 6 to 12 carbon atoms in branched chain arrangement, R<sub>1</sub> is an alkyl group containing 7 to 8 carbon atoms, R<sub>2</sub> is an alkyl group containing from 4 to 9 carbon atoms in branched chain arrangement and x is 1 or 2. This ester may comprise from about 20% up to 100% of the oil component of the grease. Preferably it comprises from about 70% to 90% of the oil component. The remainder of the oil component may suitably be a mineral oil fraction, but blends of this complex ether ester with other esters, with polymeric ethers and with other non-hydrocarbon materials of lubricating characteristics may also be employed.

We have found that greases of the above composition have valuable properties for the lubrication of ball and roller bearings over a wide temperature range which are not obtainable by greases or compositions heretofore proposed for this purpose. In addition to good low temperature torque characteristics and other superior lubricating properties at low temperatures down to about  $-60^{\circ}$  F., they also have high dropping points and provide satisfactory lubrication with negligible change in texture and consistency for long periods of time even at temperatures above  $200^{\circ}$  F. They are characterized particularly by a resistance to shear and by good stability in the presence of water.

The complex esters described above which comprise the oil component of our greases may be obtained by reacting together dicarboxylic acids, monohydric alcohols and dihydric ether alcohols

or suitable derivatives thereof according to any of the known methods for producing esters. They may conveniently be prepared by heating together a suitable dicarboxylic acid, dihydric ether alcohol and monohydric alcohol at about 150-200° C., preferably in the presence of an esterification catalyst such as a sulfonic acid or zinc chloride, and of a volatile solvent such as benzene, toluene, xylene, etc. A suitable ester of this type may be produced, for example, by heating together under reflux a mixture comprising dipropylene glycol, sebacic acid and 2-ethylhexanol in a 1:2:2 mol proportion respectively, with benzene as the solvent and with about 0.5 percent of a sulfonic acid as the esterification catalyst. The reaction is continued until an amount of water equivalent to a mol proportion of 4 with reference to the weight of the reactants is collected and the neutralization number of the product is approximately zero. The mixture is then neutralized with a mild basic reagent such as sodium bicarbonate and distilled under vacuum, removing the volatile solvent and traces of water and any excess of monohydric alcohol. As an alternate method, a polyhydric ether alcohol and dicarboxylic acid, in a 1:2 mol proportion respectively, may be permitted to react completely before the monohydric alcohol is added and the esterification then continued until all the acid groups have been esterified.

The acids which may be employed in the esterification are the saturated aliphatic dicarboxylic acids containing from 3 to 14 carbon atoms. As examples of such acids there may be mentioned particularly malonic, succinic, isosuccinic, glutaric, ethyl malonic, pyro tartaric, adipic, pimelic, suberic, azelaic and sebacic. Of these, azelaic and sebacic are particularly suitable. Mixtures of such acids may also be used.

The dihydric ether alcohols used are most suitably polyalkylene glycols containing up to 12 carbon atoms obtained by condensation in the known manner of 1,2 diols containing from 2 to 6 carbon atoms. Of these, the polypropylene glycols, particularly dipropylene glycol and tripropylene glycol, are especially suitable. Instead of a single glycol, mixtures of the above glycols may be employed.

The monohydric alcohols employed are saturated aliphatic alcohols containing from 1 to 9 carbon atoms. They are preferably branched chain non-tertiary alcohols containing from 4 to 9 carbon atoms. Suitable alcohols of this type which may be mentioned are 2-butanol, 2-ethylbutanol, 2-pentanol, 2-methylpentanol, 4-methylpentanol, 2,3-dimethylbutanol, 2-hexanol, 2-ethylhexanol, 2-heptanol, 3-heptanol, 2,3-dimethylpentanol, 4-methyl-2-pentanol, 2-octanol, 2-methyloctanol, 2-nonanol, 3-nonanol, and so forth. Such alcohols may be used either singly or as mixtures in the esterification reaction.

The sodium myristate soap which is employed as the thickening agent may be prepared by saponifying a mixture of low molecular weight fatty acids comprising at least 70%, and preferably at least 90% by weight, of myristic acid and/or the glycerides of such acids with caustic soda or other suitable sodium compound, preferably employing a small excess of the alkali sufficient to provide an excess of about 0.1 to about 1% of free alkali in the finished grease. In addition to this soap the grease may contain minor amounts of other thickening agents such as other metal soaps, polymeric materials, etc. The grease may suitably contain from about 15%

to about 25% by weight of the sodium myristate soap or of the sodium myristate soap and other thickening agents.

The greases of this invention may be prepared by conventional grease making procedures. In making a grease in which a mineral oil fraction comprises a portion of the oil base, the grease may advantageously be made by forming the soap in situ with the saponification carried out in the presence of the mineral oil component, and then finishing off with the ester component. Greases for the lubrication of high speed bearings are preferably prepared by the method described in Patent No. 2,542,570, dated February 20, 1951. In accordance with the method of said patent, a myristic acid mixture is saponified with a small excess of sodium hydroxide in the presence of small amounts of mineral oil and water, the resulting soap base dehydrated at a temperature in the range 295-320° F. and sufficient synthetic oil added to obtain the desired consistency, the synthetic oil addition being carried out in two stages so that a total amount of oil equal to at least twice the weight of the fatty acids initially charged is added before the temperature of the mass is allowed to drop below 260° F.

Various addition agents may be added in accordance with common practice in the compounding of lubricating greases, such as antioxidants and other stabilizing agents, corrosion inhibitors, extreme pressure agents, and so forth. Suitable stabilizing agents include various amines, alkylated phenols, beta-naphthol and phosphorus- and sulfur-containing compounds such as alkyl and aryl thiophosphates and their metal salts. N,N' diphenyl p-phenylene diamine has been found to be particularly effective for this purpose. It may suitably be employed in amounts ranging from about 0.1% to about 8%, and preferably from about 0.5% to about 5% by weight based on the weight of the grease. This compound may be added to the grease by any of the methods commonly employed for incorporating additives such as by adding it in the form of a slurry in a portion of the lubricating oil base or in solution in a volatile solvent, which is later flashed off. A particularly convenient method comprises adding it to the grease in the form of a solution in tricresyl phosphate. The latter serves as a solubilizing agent and carrier for the diphenyl p-phenylene diamine in addition to imparting its known anti-wear properties to the grease. A suitable composition for addition to the grease, comprising the amine and tricresyl phosphate in a ratio of about 1 to 3 by weight, may be obtained by heating them together at about 200° F.

The following example is presented to illustrate the preparation of a representative grease failing within the purview of our invention. It is understood, however, that this example is merely illustrative and not intended to limit the scope of the invention in any way.

#### EXAMPLE I

A small pestle stirred kettle was charged with 400 grams of myristic acid having a neutralization number of 240, a saponification number of 241, and a titer, °C., of 41.8, 300 grams of water and 240 grams of lubricating oil obtained by clay and solvent refining a paraffinic distillate oil. The charge was heated to 170-190° F. and 144 grams of a 50.3% aqueous sodium hydroxide, sufficient to give a slight excess, was added with stirring. After saponification the temperature

was maintained at 295-320° F. for two hours to effect dehydration while the stirring was continued. The temperature was then allowed to decrease gradually while 1620 grams of an ester were added which was obtained by reacting together sebacic acid, dipropylene glycol and 2-ethylhexanol according to the method described above for obtaining complex ether esters. Analysis showed this ester to be predominantly



The physical tests on this ester and on the mineral oil are as follows:

|                            | Ester | Mineral Oil |
|----------------------------|-------|-------------|
| Flash, COC, ° F.           | 455   | 455         |
| Fire, COC, ° F.            | 535   | 525         |
| Viscosity, SUS, at 100° F. | 240   | 332         |
| Viscosity, SUS, at 210° F. | 55    | 55          |
| Viscosity Index            | 140   | 103         |
| Pour, ° F.                 | -65   | 0           |
| Neutralization number      | 0.11  | -----       |
| Saponification number      | 277   | -----       |

The temperature of the mass was controlled during the addition of the ester so that approximately 1200 grams of the latter was added while the mass was at a temperature above 260° F. and the remainder added while the mass was at a temperature below 260° F. At a temperature below about 250° F. 23.9 grams of N,N' diphenyl paraphenylenediamine was added in the form of a solution of 67 grams of tricresyl phosphate. The product obtained was a tan short fiber grease having the following calculated composition:

|                                   | Per cent |
|-----------------------------------|----------|
| Sodium myristate                  | 18.4     |
| Mineral oil                       | 10.0     |
| Ester                             | 67.7     |
| Excess NaOH                       | 0.1      |
| N,N' diphenyl p-phenylene diamine | 1.0      |
| Tricresyl phosphate               | 2.8      |

The following table shows some of the properties of the foregoing grease comparatively with those of a sodium myristate grease of similar preparation and composition containing in place of the ester a mineral lubricating oil of the type commonly used in compounding ball and roller bearing greases. This mineral oil was a mixture of distillate and residual paraffinic oils having an SUS viscosity at 210° F. of 100.0, a viscosity index of 92, a flash point, COC of 520 and a fire point, COC, of 585.

Table I

| Grease                                               | Mineral Oil Base | Ester Base |
|------------------------------------------------------|------------------|------------|
| Dropping Point, ° F.                                 | 404              | 408        |
| Normal-Hoffman Oxidation: Pressure drop in 100 hours | 5.5              | 4.4        |
| Dynamic Shear Test;                                  |                  |            |
| Miniature penetration, before                        | 51;52            | 43;44      |
| Miniature penetration, after                         | 184;189          | 54;54      |
| Copper Corrosion Test, AN-G-5a                       | Pass             | Pass       |
| Dynamic Water Resistance, AN-G-5a: Percent Loss      | 1.3;4.0          | 3.3;4.0    |
| Low Temperature Torque (2,000 g.-cm.):               | -----            | -----      |
| Seconds/revolution at 0° F.                          | 8.4              | 8.5        |
| Seconds/revolution at -10° F.                        | 74.6             | 36.2       |
| Seconds/revolution at -20° F.                        | >120             | >120       |
| Seconds/revolution at -30° F.                        |                  | 1.8        |
| Seconds/revolution at -40° F.                        |                  | 3.8        |
| Seconds/revolution at -50° F.                        |                  | 9.8        |
| Seconds/revolution at -60° F.                        |                  | 29.4       |
| Seconds/revolution at -70° F.                        |                  | >120       |

The dynamic shear test of the foregoing table is a measure of the resistance of the grease to texture change when worked under high shearing stress, the test being carried out as described in U. S. 2,450,219, column 5, lines 6-19. A small change in miniature penetration of the sample after the test in comparison with the original is indicative of excellent texture stability under high shearing stress. The miniature penetration test is described in Ind. Eng. Chem., analytical edition, vol. II, page 108, February 15, 1939.

The low temperature torque test of the foregoing table is essentially a measure of the resistance of the grease to congealing and of its ability to afford proper lubrication under extremely low temperature conditions, such as are encountered in aircraft at very high altitudes. The apparatus employed for the test consists essentially of a vertically mounted hollow spindle with a No. 204K Conrad type 8-ball bearing mounted on the bottom, and a drum on which is wrapped a coiled line for applying torque mounted on the top. The bearing, packed with a 60% capacity charge of the grease to be tested, is clamped at the inner race to the spindle, while the outer race is clamped immovably to a stationary cup within which the bearing is inserted. The assembly is inserted with the lower bearing end in a low temperature bath containing isopropyl alcohol, and the desired temperature of the bath and bearing is attained by dropping Dry Ice in the bath. The drum and drum extension carried at the upper end of the hollow spindle and protruding from the bath are held in vertical position by a tapered roller bearing. The line coiled around the drum extends over a pulley to a container into which the desired weights are added to apply the torque load to the hollow spindle to thereby cause rotation of the spindle and inner race of the bearing with respect to the fixed outer race. A time of not less than two hours is utilized to cool the bearing to the test temperature, and an additional soaking period at the test temperature is permitted such that the test is not run until three hours from the start of cooling. When the desired bearing temperature and soaking period are attained, a 2000 gram-centimeter torque load is applied in both clockwise and counter-clockwise directions, and the number of seconds for one rotation in each direction is observed. The values obtained with rotation is clockwise and counter-clockwise directions are given separately in the table under the headings cw. and ccw., respectively.

The foregoing table shows that the ester base grease combines a high dropping point equivalent to that of the mineral oil base grease with good low temperature torque characteristics. In addition the ester base grease has a greatly improved resistance to shear as compared with the mineral oil base grease, and equally satisfactory oxidation stability, water resistance and anti-corrosiveness.

The following table shows the high temperature properties of ester base greases of this invention as compared with those of other ball and roller bearing greases containing different oil bases, soaps and additives.

7  
**Table II.—High temperature performance test**  
[300° F. and 10,000 R. P. M.]

| Grease No. | Soap Base                                                   | Oil Component        | Additive                                                  | Hours to Failure |
|------------|-------------------------------------------------------------|----------------------|-----------------------------------------------------------|------------------|
| 1          | Na Myristate                                                | Mineral Oil          | None                                                      | 219              |
| 2          | do                                                          | do                   | 1% Diphenylamine                                          | 392              |
| 3          | do                                                          | do                   | 1% Triphenylguanidine                                     | 452              |
| 4          | do                                                          | do                   | 1% Diphenyl p-phenylene diamine                           | 1,056            |
| 5          | do                                                          | do                   | 1% Diphenyl p-phenylene diamine +2.8% tricresyl phosphate | 1,308            |
| 6          | Na 4:1 Stearic acid: Tallow                                 | do                   | None                                                      | 273              |
| 7          | Li 3:1 Hydrogenated castor oil: Triple pressed stearic acid | do                   | do                                                        | 144              |
| 8          | Na 3:1 Menhaden oil: Snodotte acids 5% Al Stearate          | do                   | 1% Diphenylamine +3% Sulfonic acids                       | 254              |
| 9          | Li Hydrogenated Fish Oil                                    | Silicone fluid       | None                                                      | 262              |
| 10         | Na Myristate                                                | Butyl stearate       | 1% Diphenylamine                                          | 264              |
| 11         | do                                                          | Tetradecyl sebacate  | do                                                        | 572              |
| 12         | do                                                          | Diocetyl phthalate   | do                                                        | 396              |
| 13         | do                                                          | Polymerized ether    | do                                                        | 156              |
| 14         | do                                                          | Chlorinated diphenyl | 2.8% Diphenylamine                                        | 61               |
| 15         | do                                                          | Ether ester          | 1% Diphenylamine                                          | 843              |
| 16         | do                                                          | do                   | 0.9% Triphenylguanidine                                   | 1,106            |
| 17         | do                                                          | do                   | 1% Diphenyl p-phenylene diamine +2.8% tricresyl phosphate | 2,376            |

All of the sodium myristic greases of the above table were prepared according to the procedure described in Example I. Grease No. 17 is the grease prepared in Example I, and Greases No. 15 and 16 differ from this grease only in the additives employed. Grease No. 5 is the mineral oil base grease of Table I. Grease No. 9 is a commercial grease generally rated as a very superior grease for the lubrication of high speed ball bearings over a wide temperature range. Analysis of this grease indicates that it is composed of 23% of a lithium soap of hydrogenated fish oil fatty acids, 0.2% free fatty acid and a silicone fluid of an SUS viscosity of 330 at 100° F. This grease has a dropping point of 422° F. and gave 33.4 seconds/revolution at -40° F. in the low temperature torque test.

The high temperature performance test of the foregoing table is a test for determining the performance characteristics of greases in anti-friction bearings at elevated temperatures and high rotative speeds. The test unit consists essentially of a steel spindle supported on ball bearings in an electrically heated housing and driven by an electric motor connected into an electric circuit containing a low amperage fuse 0.1 ampere below that required for full load running. The bearings are Norma-Hoffman ABEC No. 3 grade, and are mounted on the spindle approximately 5 1/8 inches apart. A thrust load of 17.5 pounds is applied to the bearings. One bearing is used for test purposes and the second bearing, which is not heated, is used as a guide bearing. The test consists of operating the test bearing for twenty-four hours at 10,000 R. P. M. and at a temperature of 300° F. followed by a shut down and cooling period of two hours, and repeating this cycle until the lubricant fails, which is indicated by rupture of the low amperage fuse in the motor circuit. In starting up the test, three grams of the test grease are charged to the test bearing and worked into and around the races and balls. The bearing is next rotated both clockwise and counterclockwise for one minute each at 200 R. P. M. and assembled into the test unit. The heaters and the motor are then started and the test bearing brought up to the test temperature as rapidly as possible, which requires 1.0 to 1.25 hours, while the spindle is rotated at a speed of 10,000 R. P. M. After 24 hours of operation the heaters and motors are

25 shut off for 2 hours, during which the temperature of the test bearing drops to a minimum of 120-130° F. The total hours of operation, excluding the two hour shutdown periods, to the failure point is recorded as the "hours to failure."

30 A grease giving satisfactory lubrication for 1000 hours at 300° F. under the conditions of this test is considered a very superior lubricant for the lubrication of anti-friction bearings at elevated temperatures and at high rotative speeds.

35 As shown in the tables, the greases of our invention are markedly superior in both high and low temperature properties to greases comprising other soap and oil base combinations, including the usual types of soaps with mineral oils, and sodium myristate with both mineral oils and with other types of synthetic non-hydrocarbon oils such as have been proposed heretofore as lubricating oil bases. More particularly, the greases of our invention are superior for lubricating small, light, high speed bearings, such as those used in aircraft gyroscopes, over a wide range of temperatures.

45 Obviously many modifications and variations of the invention, as hereinbefore set forth, may be made without departing from the spirit and 50 scope thereof, and therefore only such limitations should be imposed as are indicated in the appended claims.

We claim:

55 1. A wide temperature range ball and roller bearing grease consisting essentially of an oleaginous liquid lubricating base and a thickening agent comprising in major proportion sodium myristate, said oleaginous liquid lubricating base comprising in substantial proportion a complex polyester of lubricating characteristics represented by the general formula



60 wherein R is an aliphatic ether group containing from 4 to 12 carbon atoms, R<sub>1</sub> is an alkyl group containing from 1 to 12 carbon atoms, R<sub>2</sub> is an alkyl group containing from 1 to 12 carbon atoms and x is an integer from 1 to 5.

65 2. The grease composition of claim 1 wherein the complex polyester is represented by the general formula



70 wherein R is an aliphatic ether group containing

from 6 to 12 carbon atoms in branched chain arrangement,  $R_1$  is an alkyl group containing from 7 to 8 carbon atoms,  $R_2$  is an alkyl group containing from 4 to 9 carbon atoms in branched chain arrangement and  $x$  is an integer from 1 to 2.

3. The grease composition of claim 1 wherein the complex polyester is a compound having the formula



4. The grease composition of claim 1 containing a small amount of free alkali.

5. The grease composition of claim 1 in which the complex polyester is obtained by reacting together under esterification conditions a polypropylene glycol containing from 6 to 9 carbon atoms, sebacic acid and 2-ethyl hexanol. 15

6. The grease composition of claim 1 containing 0.1-8% by weight of  $N,N'$  diphenyl para-phenylene diamine.

7. The grease composition of claim 1 containing 0.5-5% by weight of  $N,N'$  diphenyl para-phenylene diamine.

8. The grease composition of claim 1 in which the oleaginous liquid lubricating base comprises a minor proportion of a mineral oil of lubricating characteristics.

9. The grease composition of claim 1 containing 0.3-15% by weight of tricresyl phosphate.

10. A lubricating grease consisting essentially of an oleaginous liquid lubricating base, about

15-25% by weight based on the grease of a sodium soap of a soap-forming fatty material containing at least 70% based on the fatty material of myristic acid, 0.5-5% by weight of  $N,N'$  diphenyl p-phenylene diamine, 1.5-15% by weight of tricresyl phosphate and 0.1-1.0% of free alkali, said oleaginous liquid lubricating base comprising in minor proportion a mineral lubricating oil and in major proportion a complex polyester of lubricating characteristics obtained by reacting together under esterification conditions a polypropylene glycol containing from 6 to 9 carbon atoms, sebacic acid and 2-ethyl hexanol.

JOHN P. DILWORTH.  
CHARLES H. CULNANE.

References Cited in the file of this patent

UNITED STATES PATENTS

| Number    | Name           | Date           |
|-----------|----------------|----------------|
| 2,436,347 | Zimmer et al.  | Feb. 17, 1948  |
| 2,448,567 | Zisman et al.  | Sept. 7, 1948  |
| 2,450,221 | Ashburn et al. | Sept. 28, 1948 |
| 2,497,432 | Blake          | Feb. 14, 1950  |
| 2,499,984 | Beavers et al. | Mar. 7, 1950   |
| 2,539,503 | Zisman et al.  | Jan. 30, 1951  |
| 2,542,570 | Puryear et al. | Feb. 20, 1951  |

OTHER REFERENCES

30 Hain et al., Synthetic Low Temperature Greases from Aliphatic Diesters, article in Industrial and Eng. Chem., vol. 39, pp. 500-506, April 1947.